

Sept. 16, 1924.

1,508,720

L. M. PERRY

FINISHED SHEET MATERIAL AND METHOD OF FINISHING THE SAME

Filed July 1, 1922



Invantor:  
Lloyd M. Perry,  
Wayne Brook Janney Valley  
Hills.

Patented Sept. 16, 1924.

1,508,720

# UNITED STATES PATENT OFFICE.

LLOYD M. PERRY, OF NASHUA, NEW HAMPSHIRE, ASSIGNOR TO NASHUA GUMMED & COATED PAPER COMPANY, OF NASHUA, NEW HAMPSHIRE, A CORPORATION OF MASSACHUSETTS.

## FINISHED SHEET MATERIAL AND METHOD OF FINISHING THE SAME.

Application filed July 1, 1922. Serial No. 572,279.

To all whom it may concern:

Be it known that I, LLOYD M. PERRY, a citizen of the United States, and a resident of Nashua, in the county of Hillsborough and State of New Hampshire, have invented an Improvement in Finished Sheet Material and Methods of Finishing the Same, of which the following description, in connection with the accompanying drawings, is a specification, like characters on the drawings representing like parts.

The object of this invention is to provide an improved method of surface-finishing paper or other sheet material and an improved product which avoids certain disadvantages inherent in the processes heretofore employed.

The common method of producing a glazed finish surface on paper has been first to cover the paper with a surface-coating containing a wax emulsion, the latter being prepared from carnauba wax, beeswax, ceresine or other wax or oil capable of emulsification when heated with dilute alkaline solution or with alkaline solution and soap. In the case of coated paper this emulsion is mixed with the coating compound and applied to the surface of the paper. After being dried it is passed through a friction calender and subjected to the burnishing action of the calender rolls.

It is difficult, however, completely to emulsify the wax or completely to maintain it emulsified. Relatively large particles of free wax are apt to be present causing streaks or spots on the paper under the action of the friction calender. The alkali required to insure emulsification of the wax is also apt to affect the shades in certain dyes and pigments. These and other difficulties I have found can be avoided by using as a substitute for the wax emulsion an insoluble metallic salt of a fatty acid, such as zinc stearate.

The invention will be best understood by reference to the following description when taken in connection with the accompanying illustration showing one method of applying the coating and finishing the paper, the scope of the invention being more particularly pointed out in the appended claims.

In the drawings,—

Fig. 1 is a diagrammatic representation

of the apparatus commonly employed in 55 coating sheet paper; and

Fig. 2 is a diagrammatic representation of a calender machine for imparting a surface finish to the paper after it has been 60 coated by my improved process.

In carrying out my invention I employ a certain amount of an insoluble metallic salt of a fatty acid, such as zinc stearate. The latter can be obtained in either dry, or in pulp form having approximately 75% 65 water.

Zinc stearate in dry form is difficult to incorporate with the coating compound, and prior to such incorporation must be made into a smooth paste with water; preferably 70 to the paste thus formed, there is added a certain amount of sulphonated oil, such as Turkey red oil, in the approximate proportion of three pints of oil to thirty pounds of dry zinc stearate. This produces a paste 75 of smoother consistency.

Zinc stearate in pulp form is more easily incorporated with the coating mixture, but more or less water is apt to evaporate from the pulp form during storage, so that with 80 the dry form a coating mixture of more accurate proportions may be prepared.

The paste thus prepared from dry zinc stearate, or the zinc stearate in pulp form 85 (used directly) may be used very much as the wax emulsion referred to has heretofore been used, although it is necessary to add only about one-half as much (on a dry basis) of the zinc stearate as in the case of 90 the wax emulsion.

In preparing the coating, the coating mixture is first mixed as heretofore. The zinc stearate paste, prepared as described, is then added to the coating mixture and mixed thoroughly in an ordinary mixing machine. The amount of zinc stearate to be added to the coating mixture should preferably be about 1 1/4 to 3% (on a dry basis) of zinc stearate in the total coating mixture, dependent 95 on the nature of the coating with which it is used. When the color mix has had the zinc stearate thoroughly intermingled, there should be added to the completed mixture a quantity of some suitable sizing, such as casein. The quantity will vary with the nature of the coating but ordinarily will be approximately from 10 to 12%. The amount 100 of water in the color mix will vary with the

pigment used. When the coating is thus finally prepared the zinc stearate or other salt employed is in a finely divided solid form thoroughly incorporated in the color mix.

The coating thus prepared may be applied to the paper in any suitable manner, as for example, by the apparatus shown diagrammatically in Fig. 1. Herein, the coating mixture 3 is contained within the tank 5, within which operates the roller 7 immediately beneath the guide drum 9. The paper feed roller 1 supplies the paper to the guide drum 9 over the guide rolls 13 and at the drum 9 it has applied to it a suitable amount of coating mixture by means of a brush 15 which rotates in contact with the tank roller 7 and the paper sheet 17. The coating thus applied to the paper sheet is smoothed and distributed by any suitable means, as by means of the stationary brush 19, engaging the paper while still on the cylinder, and a series of brushes 21 which may be either stationary or movable engaging the paper sheet where it passes over the rubber apron 23. The sheet then passes to a suitable drying apparatus which is indicated conventionally only at 25, where it is hung in festoons and subjected to the necessary drying action, whence it passes to and is wound upon the storage drum 27.

To give the paper sheet its surface finish it may be subjected to any suitable finishing action, such as that of a friction calender, a super-calender, a flint machine, or a brush machine. Herein for illustrative purposes, there is diagrammatically shown in Fig. 2 a friction calender having the calender rolls 29 and 31. The roll 29 may be of steel with a hard smooth surface and interiorly heated. It is adjustably pressed against the lower roll 31, the latter having a relatively yieldable surface such as is presented by rings of compressed cotton. The cotton surfaced roll 31 is driven by frictional contact with the underlying smooth steel roll 32 at the same speed as that of the roll 32 and at a somewhat lesser speed than that of the roll 29. The paper passes from the roll 27, where it is subjected to a drag or braking action, through the calender rolls to the roll 33 on which it is wound up for storage or shipment. The coating thus applied and containing the zinc stearate responds readily to the burnishing action of the calender rolls and gives a high finish without certain of the defects involved in the use of wax emulsion.

Through the use of an insoluble metallic salt of a fatty acid, such as zinc stearate, a coating substantially invariable in its composition may be applied. In the use of wax emulsions for this purpose there is not only an unavoidable variation in the quality of the wax and in the strength of the alkali,

but a variation due to the personal factor in preparing it. Carnauba wax and beeswax also contain impurities, whereas zinc stearate and all the insoluble salts of fatty acids may be obtained as substantially chemically pure products. Zinc stearate, furthermore, is very white, giving a lighter shade to the coating and permitting a brighter color to be obtained than in the case of wax emulsions which tend to give the paper a yellowish tinge. The melting point of zinc stearate, and of a number of other insoluble salts of fatty acids, is relatively high as compared with the melting point of the waxes commonly employed, so that, when used with white or light colored coatings, where opacity is desired, the opacity of the coating is preserved, whereas in the case of the wax emulsions the coating tends to become more or less transparent under the action of the friction calender. In cases where this opacity is not desired, an insoluble salt of a fatty acid having a lower melting point may be employed, such, for example, as an oleate or a mixture of an oleate and a stearate.

The quality of the paper finished by zinc stearate is as good or better than that finished by the best wax, while the cost of the zinc stearate is no more than that of the cheapest wax employed and about half as much as that of the best wax. Wax emulsions are also sensitive to impurities such as mineral salts in the color mix and the emulsions are apt to be broken down thereby, causing imperfection in the finished paper. The excess of alkali commonly present in wax emulsions also has a tendency to render fugitive the shades of many dyes and pigments employed. Zinc stearate, however, and other insoluble salts of fatty acids, are not readily influenced by substances used in the color mix and, on the other hand, have no effect on those shades which are rendered fugitive by the excess of alkali. Nor does it have any tendency to cause foaming under the brushes which is a common occurrence in the use of wax emulsion, due chiefly to the presence of soap in the emulsion.

The paper coated with the use of zinc stearate also has a softer quality and lacks the harshness of paper finished through the use of wax emulsion.

A glazed finished waterproofed paper in which the waterproofing agent is casein, shellac or other materials soluble in dilute alkali is more waterproof when made with zinc stearate than when made with wax emulsion, since the latter commonly contains an excess of fixed alkali which impairs the water resistance of the waterproofing agent; whereas zinc stearate is free from such alkali.

The invention is particularly applicable

to glazed coated paper finished on the friction calender, but is also usable for finishing coated paper by means of flint machines, super-calenders and brush machines. It 5 may also be advantageously used in the surface finishing of sheet material other than paper or of paper products which are not commonly termed "coated", such, for example, as so-called high finished press-board.

10 While I have herein shown and described for purposes of illustration one specific embodiment of the invention, it is to be understood that the same is not limited to the particular detailed steps or substances herein referred to, but that extensive deviations 15 may be made therefrom without departing from the spirit thereof.

Claims:

1. The method of surface finishing paper 20 or the like which consists in preparing a liquid coating mixture including a pigment mixed with from  $1\frac{1}{4}$  to 3 per cent of zinc stearate, applying said solution to the surface of the paper, drying the same, and 25 subjecting it to the burnishing action of a finishing agent to produce a surface glaze thereon.

2. The method of surface finishing paper or the like which consists in preparing a liquid coating mixture including a pigment 30 and zinc stearate, applying said mixture to the surface of the paper, drying the same, and subjecting it to the burnishing action of a finishing agent to produce a non-transferable adherent glaze. 35

3. The method of surface finishing sheet material which consists in preparing a liquid coating mixture containing an insoluble salt of a fatty acid in finely divided solid form and capable of producing a glazed surface 40 under a finishing action, applying said mixture to the surface of the material, drying the same, and subjecting it to the action of a finishing agent to produce a non-transferable, closely adherent, glazed coating. 45

4. A surface coated, glazed paper having a surface coating only of a closely adherent and a permanent non-transferable glaze, the latter containing an insoluble salt of a fatty acid. 50

In testimony whereof, I have signed my name to this specification.

LLOYD M. PERRY.